

1

2,756,148

## PHOTOGRAPHIC EMULSION HAVING CLAYDEN EFFECT SUSCEPTIBILITY

Edgar A. MacWilliam, Rochester, N. Y., assignor to Eastman Kodak Company, Rochester, N. Y., a corporation of New Jersey

No Drawing. Application June 29, 1954,  
Serial No. 440,282

9 Claims. (Cl. 95—7)

This invention relates to photography and particularly to a method of making a photographic emulsion which shows high susceptibility to the Clayden effect.

It has been shown that the sensitivity of some photographic materials when exposed by a relatively long duration exposure may be reduced if the materials have first been exposed to illumination of short duration, i. e. 0.001 second or less. This effect has been called the Clayden effect. The feature which characterizes the Clayden effect is that the initial exposure of short duration to relatively high intensity light desensitizes the emulsion so that subsequent exposure to weak intensity light produces less effect than if the pre-exposure had not been given. As usually observed the density resulting from the two superposed exposures is less than that of the single exposure to the low intensity light on making it appear that the effect is a reversal.

The effect known as the Clayden effect has a number of practical applications. Yule and Maurer have described in their application Serial No. 291,623, now U. S. Patent No. 2,691,586, use of the Clayden effect in preparing a pre-screened photographic material with which halftone negatives may be prepared from a continuous tone positive without the use of the conventional halftone screen. The usefulness of such pre-screened materials in the graphic arts for letterpress, lithographic and intaglio printing depends on the degree of desensitization obtainable and hence, on the degree of sensitivity of the material to the Clayden effect.

It is, therefore, the principal object of my invention to provide a method for improving or increasing the susceptibility of a photographic emulsion to the Clayden effect. Other objects will appear from the following description of my invention.

These objects are accomplished and the susceptibility of the photographic emulsion to Clayden desensitization is enhanced, by precipitating a silver chlorobromide in gelatin in such way as to form first a relatively chloride-rich precipitate which is subsequently converted to a bromide-enriched silver chlorobromide by addition of bromide ions during at least the latter part of the precipitation cycle, preferably during at least the last  $\frac{1}{3}$  of the precipitation cycle of the emulsion making procedure. The emulsions ranging from 40 mole percent chloride and 60 mole percent bromide to 90 mole percent chloride and 10 mole percent bromide have been found to be the most useful. I have also found that it is advantageous to precipitate the silver chlorobromide at higher temperature than normally used, that is, that the susceptibility to the Clayden effect increases with increasing temperature of precipitation of the silver halide.

Where I refer to addition of bromide ions or addition of alkali metal bromide to the emulsion "during at least the latter part" of the precipitation cycle, I mean that the alkali metal bromide is added during or after the silver salt is added or during the entire cycle, as long as substantially no silver salt is added after the addition of the alkali metal bromide is complete. It has been found that

2

as the time of the addition of the alkali bromide is decreased, the susceptibility of the emulsion to the Clayden effect is increased.

Instead of forming a bromide-enriched silver chlorobromide as described above, it is also possible to make a silver chlorobromide or silver chloride precipitate and subsequently convert the surface of the grains thus formed to silver bromide. Useful silver chlorobromide emulsions can be made by this technique having a chloride content ranging from 40 to 60 mole percent.

According to my preferred method of making a photographic emulsion, a gelatin solution of an alkali metal chloride and an alkali metal bromide is first prepared, in which the solution contains more than about one-half molar proportion of the alkali metal chloride and less than 0.1 molar proportion of the alkali metal bromide. The alkali metal halides customarily used are the sodium, potassium or ammonium salts. The concentration of alkali metal halide in the gelatin may vary considerably; however, the range from 0.4 gram to 3.0 grams of alkali metal halide per gram of gelatin has been found to give satisfactory results.

To a gelatin solution of alkali metal halide there is added during a definite period of time of from two to ten minutes a solution of one molar proportion of silver nitrate in distilled water. The solution is stirred during the entire addition of the silver nitrate, and during at least the latter part of said addition of silver nitrate, an additional amount, less than one-half molar proportion but more than  $\frac{1}{10}$  molar proportion of alkali metal bromide is added to the emulsion. Preferably during the addition of the alkali metal halides, these halides are kept in excess of the silver salt; however, this is not essential. As a final step, unreacted soluble salts are removed from the emulsion either by washing in the customary way or by coagulating the emulsion with a suitable gelatin coagulant, e. g., sodium sulfate, which removes the gelatin and silver halide from the solution.

I have found that the precipitation of the silver halide should be carried out at a temperature of from 50° to 95° C. in order to obtain the enhanced Clayden effect susceptibility. A temperature of approximately 70° C. is preferred.

After addition of the second portion of alkali metal bromide, I prefer to stir the emulsion for an additional time of about ten minutes at approximately 70° C. and remove soluble salts, then sensitize the emulsion with a sulfur sensitizer customarily used such as disclosed in Sheppard U. S. Patent 1,574,944, then add additional gelatin and stir the emulsion for an additional time, approximately 30 minutes, after which it is cooled.

The emulsion may be sensitized with an optical sensitizing dye of the merocyanine or hemioxonol class as described in my application Serial No. 440,283, filed concurrently herewith, and this also increases the Clayden effect susceptibility.

My invention will be further described by reference to the following examples in which the materials and conditions are merely illustrative, the invention being limited only by the scope of the appended claims.

Example 1

A solution of 170 grams of silver nitrate in 650 cc. of distilled water at 60° C. was added during 6 $\frac{1}{3}$  minutes to a solution of 50 grams of gelatin, 42 grams of sodium chloride and 1.75 grams of potassium bromide in 1287 cc. of distilled water at 71° C. Four and one-quarter minutes after the commencement of the silver nitrate addition, the addition of a solution of 37 grams of potassium bromide in 127 cc. of distilled water at 40° C. was begun and continued for the remaining two minutes of the silver run. The resulting emulsion was stirred

for 10 minutes at 71° C. before the addition of 25 grams of dry gelatin soaked in water. The emulsion was stirred a further four minutes at 71° C. and was then cooled to 29° C. Sufficient saturated sodium sulfate solution was added to cause the emulsion to coagulate and settle out (about 300 cc.). The emulsion cake was rinsed three times with chilled water and then dispersed in water at 40° C.

The emulsion was sensitized with a sulfur sensitizer such as disclosed in Sheppard U. S. Patent 1,574,944 to its maximum contrast. A further portion of 86 grams of gelatin was then added and stirred until it was dispersed. Before coating there was mixed with the emulsion from 0.1 to 0.2 gram of 1-carboxymethyl-5-[(3-ethyl-2-(1-benzoxazolylidene)-ethylidene)-3-phenyl-2-thiohydantoin dissolved in 1% alcoholic triethylamine solution.

In order to test the Clayden effect susceptibility the emulsion after coating was exposed through a step tablet with 0.15 density increments to illumination from a Kodatron flash lamp at 60 inches. The emulsion was then exposed through a similar step tablet set at right angles to the first to lower intensity illumination for 0.1 second. The emulsion was then developed for 2½ minutes at 68° F. in a developer of the following composition:

|                             | grams |
|-----------------------------|-------|
| Hydroquinone                | 22.5  |
| Sodium sulfite (desiccated) | 30    |
| Parafomaldehyde             | 7.5   |
| Potassium metabisulfite     | 2.6   |
| Boric acid, crystals        | 7.5   |
| Potassium bromide           | 1.6   |
| Water to 1 liter            |       |

Results were as follows:

|       | g. Dye/Mol Ag halide | Desens.<br>ΔLog E<br>Measured<br>at a Den-<br>sity of 1.0 |
|-------|----------------------|-----------------------------------------------------------|
| 0.100 |                      | 1.05                                                      |
| .150  |                      | 1.05                                                      |
| .200  |                      | >1.9                                                      |

### Example 2

Three chlorobromide emulsions were made as described in Example 1 except that the temperatures of precipitation of the silver halide were 55° C., 71° C. and 78° C. respectively, and the emulsions were coated with 0.1 g. of sensitive dye. Upon testing the coatings as described in Example 1, the extent of Clayden effect desensitization increased as the temperature of precipitation was increased, as shown in the following table:

|        | Temperature of Precipitation | Desens.<br>ΔLog E<br>Measured<br>at a Den-<br>sity of 1.0 |
|--------|------------------------------|-----------------------------------------------------------|
| 55° C. |                              | 0.10                                                      |
| 71° C. |                              | 1.05                                                      |
| 78° C. |                              | 1.20                                                      |

### Example 3

Three chlorobromide emulsions were made as described in Example 1 except that the second potassium bromide solution was added during the last six minutes, the last four minutes and the last two minutes, respectively, of the silver nitrate run, so that the silver and bromide runs ended at approximately the same time. Upon testing the coatings as described in Example 1, susceptibility to Clayden effect was found to be increased as more of the additional potassium bromide was added

4  
during the latter part of the run, as shown in the following table:

| 5        | Time of Bromide Addition | Desens.<br>ΔLog E<br>Measured<br>at a Den-<br>sity of 1.0 |
|----------|--------------------------|-----------------------------------------------------------|
| 6minutes |                          | 0.40                                                      |
| 4minutes |                          | 1.05                                                      |
| 2minutes |                          | 1.70                                                      |

What I claim is:

1. The method of making a photographic emulsion having a high susceptibility to Clayden desensitization, which comprises adding one molar proportion of a soluble silver salt to a gelatin solution of more than about one-half molar proportion of a soluble chloride and less than about 0.1 mole of a soluble bromide, with stirring, during less than ten but more than two minutes, and during a period of time beginning after the commencement of said addition of silver salt, adding an additional amount, less than one-half molar proportion but more than 0.1 molar proportion, of a soluble bromide to said solution.

2. The method of making a photographic emulsion having a high susceptibility of Clayden densensitization, which comprises adding one molar proportion of silver nitrate to a gelatin solution of about three-fourth molar proportion of an alkali metal chloride and about 0.01 molar proportion of an alkali metal bromide, with stirring, during about ten minutes, and during about the latter part of said silver nitrate addition, adding an additional approximately one-third molar proportion of alkali metal bromide to said solution, and removing unreacted soluble salts from said emulsion.

3. The method of claim 1, in which the addition of the alkali metal halides is carried out at approximately 50° C. to 95° C.

4. The method of claim 1, in which the addition of the alkali metal halides is carried out at approximately 70° C.

5. The method of claim 1, in which addition of silver nitrate is made during six minutes, and addition of alkali metal bromide is made during the last five minutes of the silver nitrate addition.

6. The method of claim 1, in which the emulsion is stirred for an additional ten minutes at approximately 70° C. after addition of the second alkali metal bromide, additional gelatin is then added, and the emulsion is stirred for an additional four minutes and then cooled to approximately 30° C.

7. The method of claim 1, in which the emulsion is cooled to approximately 30° C. after addition of the second alkali metal bromide, and is then coagulated with sodium sulfate, rinsed with water, and dispersed in water.

8. The method of claim 1, in which the final emulsion is sensitized with a sulfur sensitizer.

9. The method of claim 1, in which the final emulsion is sensitized with 1-carboxymethyl-5-[(3-ethyl-2-(1-benzoxazolylidene)-ethylidene)-3-phenyl-2-thiohydantoin.

### References Cited in the file of this patent

### UNITED STATES PATENTS

65 1,574,944 Sheppard ----- Mar. 2, 1926

### FOREIGN PATENTS

545,944 France ----- Aug. 5, 1922

580,173 Great Britain ----- Aug. 29, 1946

690,997 Great Britain ----- May 6, 1953

### OTHER REFERENCES

Wall: Photographic Emulsions (1929). Pub. by American Photographic Pub. Co., Boston (pages 98 and 75 99).